

Jan. 15, 1963

O. W. AHMANSSON ET AL

3,072,985

METHOD FOR VACUUM CASTING OF STEEL

Original Filed July 31, 1958



## 1

3,072,985

**METHOD FOR VACUUM CASTING OF STEEL**  
 Olov Wood Ahmannsson, Goteborg, and Lars Olof Uhrus,  
 Hofors, Sweden, assignors to Aktiebolaget Svenska  
 Kullagerfabriken, Goteborg, Sweden, a corporation of  
 Sweden

Continuation of application Ser. No. 752,293, July 31,  
 1958. This application Feb. 3, 1960, Ser. No. 6,568  
 4 Claims. (Cl. 22—215)

This invention relates broadly to casting of metals and more specifically to casting of metals in vacuum.

In casting steel or other metal in vacuum, the procedure is generally as follows: The molten metal passes from a receptacle, a so-called ladle, in a jet or stream down into a chiller which is located in a receiving receptacle. With the aid of suitable pumps the right amount of vacuum is created in the receptacle, for which purpose a vacuum-tight cover is arranged between the ladle and the receptacle. If proper vacuum is to be obtained, it is important, among other things, that the receptacle contains no porous material in which gas can be occluded in surface and pores.

Previously in vacuum casting steel, for example, there was no advantage in using the hot tops generally used when casting in a chiller, which are made of fire-proof material with the lowest possible capacity for heat-conduction, since these materials are always porous and have an unfavorable effect on the vacuum treatment, in that it takes a very long time to remove the quantities of gas present in the pores of the material. The quantity of gas emitted from the fire-proof material is increased by the moisture always remaining in the material. The unfavorable effect of the fire-proof material is accentuated if the material is heated, for instance, when molten metal comes in contact with the material.

The present invention relates to a process for vacuum casting steel in a chiller, and has as a primary object elimination of the difficulties associated with the use of fire-proof material for insulating the top part of the ingot in connection with the vacuum treatment of molten metal. The object of the invention is chiefly attained by the fact that during the casting process the chiller is provided with a removable upper part of non-porous material, preferably of the same material as the chiller, such as cast iron and which, after the molten metal is suitably cooled, is replaced by a suitable layer or protective hood or the like covering the top part of the ingot or casing, the layer being of porous thermoprotective material.

Additional objects and advantages of the invention will be more fully appreciated from the following detailed description of embodiments thereof, when taken together with the accompanying drawings, in which:

FIG. 1 is a schematic view of one form of apparatus for vacuum casting of metal;

FIG. 2 is a fragmentary sectional view of a chiller mold with non-porous top part;

FIG. 3 is a fragmentary sectional view corresponding to FIG. 2 with a non-porous top part replaced by a thermo-protective top;

FIG. 4 is a fragmentary sectional view or a modification having the top part enclosed in an outer steel casing;

FIG. 5 is a fragmentary sectional view corresponding to FIG. 4 with the top part replaced by a thermo-protective covering;

FIG. 6 is a fragmentary view partly in section of a further modification incorporating means for introducing exothermal reactant material to the ingot;

FIG. 7 is a fragmentary view partly in section of a further modification including heating means for the casting top;

FIG. 8 is a fragmentary view partly in section of a

## 2

further modification incorporating different heating means; and

FIG. 9 is a view taken on line 9—9 of FIG. 8.

Referring to the drawings, a usual type of chiller mold 10 is mounted on a base 12 within a lower portion of a receiving receptacle 14. Means are provided for closing and sealing the upper end of the receiving receptacle and as shown may include a casing 16 formed as a portion of a ladle 18 of any known type having a molten metal discharge spout 20. Co-acting flanges 22 and 24 on the members 16 and 14 respectively serve to establish a vacuum tight interior for the receiving receptacle. A vacuum pump 26 operatively associated with a motor 28 acting through pipe 30 and valve 32 function to create the desired amount of vacuum in the receiving receptacle.

In accordance with the present invention the chiller mold 10 is provided, before casting of the metal, with a top part 34 of non-porous material, preferably of the same material as a chiller mold, such for example as cast iron. This top 34 is designed substantially like a conventional hot top, that is, tapering upwards or narrowing toward its upper end. Hooks 36 or the like are provided for facilitating movement of the top. During the casting process the chiller mold after being placed in the receiving receptacle is provided with the top part 34 in place. A vacuum is then drawn in the receptacle and molten metal discharged into the chiller mold. When the vacuum treatment of the molten metal has been completed, when the chiller is filled, the receiving receptacle is connected with ambient air through the valve 32 which serves at the same time to cut off the vacuum pump from connection with the receptacle.

As soon as possible, that is when a thin layer of hardened material has formed against the top part 34, this top part is removed from the chiller mold. Immediately following this, a covering for the upper part of the casting is provided. In the embodiment shown in FIG. 3 this includes a cylindrical shaped casing 38 which rests on the top surface of the chiller mold and has a cross section such that a considerable gap remains between the casting shown at 40 and the inner surface of this casing 38. The space is quickly filled with a suitable thermo-protective material 42, for example kieselguhr powder, which material should also cover the top surface of the ingot or casting in order to retain the heat as long as possible.

The modification shown in FIGS. 4 and 5 differs from that shown in FIGS. 2 and 3 in that a casing 44 is fitted around the top part of the chiller mold 10 prior to the casting process and can if desired be secured to the mold. At a suitable time during cooling of the metal, it is thus only necessary to lift off the top part 34 and fill the ring shaped space thus formed between the casing 44 and the ingot or casting 40 with suitable thermo-protective material 42 which, as in the previous embodiment, preferably should cover the top surface of the casting or ingot.

The top part or cover 34 can if desired be connected with the ladle directly so that the chiller and cover together form the receiving receptacle. It would thus not be necessary to use a special or additional receiving receptacle and the volume which must be evacuated will be reduced to a minimum. For this purpose the top part would be provided with an evacuation opening and the necessary seals.

The sheet iron cover and the loose film of kieselguhr powder can be replaced by other suitable insulating films or covers, such as a finished and suitably-tapered hood, closed at the top, and which is placed over and around the top of the casting or ingot after the non-porous top part has been removed.

In FIG. 6 such a hood is shown at 46 and is suitably

designed so that an interspace is formed between it and the top part of the ingot. It is advisable to have a supply of heat in this space. As an example, holes in the top of the hood permit introduction of an exothermal mixture from a header 52 connected through a conduit 54 to a suitable source. After the hood has been placed over the ingot, a reaction is thus started when the mixture contacts the ingot which is still glowing at the top.

Another method of supplying heat to the top of the ingot is shown in FIG. 7, where a hood 56 is provided internally with a resistance heating element 58 of any desired known type such as embedded in porcelain 60, the inner surface of which is spaced from the ingot as shown at 62. This arrangement additionally permits preheating the hood 56 before it is placed over the ingot.

In FIGS. 8 and 9, a further type of hood 64 is shown having inlet burner jets 66 arranged tangentially with respect to the hood for the introduction into space 68 of gas or oil. These jets are arranged near the lower edge of hood 64 and exhaust gases can be drawn off through opening 70 in the top 72 of the hood.

In accordance with the present invention it is possible to obtain satisfactory insulating of the top part of the ingot or casting during the principal part of the period required for the complete hardening of the ingot and prevent any porous material from being in the receiving receptacle during the vacuum treatment. Additionally, no molten metal can get in contact with the fire-proof material in the vacuum chamber itself.

Manifestly minor changes can be effected in the method and described apparatus without departing from the scope and spirit of the invention as defined in the appended claims.

This application is a continuation of our application Serial No. 752,293, filed July 31, 1958, now abandoned.

We claim:

1. A method of casting metal which comprises introducing molten metal to an upright mold of non-porous

material having a removable, open-ended upper portion located within an evacuated chamber, removing said upper portion of said mold to expose the upper end of said cast metal as soon as a thin layer of solidified metal has formed against the upper portion of said mold, and immediately surrounding the exposed upper end of said cast metal with porous heat-insulating material, while maintaining said cast metal in the lower portion of said mold in the position initially assumed with respect thereto as when initially cast in said mold, and completing solidifying said cast metal, said porous heat-insulating material being applied to the exposed end of said cast metal after admission of air to said chamber.

2. The method according to claim 1, wherein said porous heat-insulating material is maintained in surrounding relationship with the exposed metal by means of a jacket.

3. A method according to claim 2, wherein the jacket is applied to the mold only after the upper non-porous part of the mold has been removed.

20 4. The method according to claim 2 wherein said jacket comprises an integral part of the lower portion of said mold.

#### References Cited in the file of this patent

#### UNITED STATES PATENTS

|           |               |               |
|-----------|---------------|---------------|
| 1,431,804 | Howard et al. | Oct. 10, 1922 |
| 1,978,996 | Gathmann      | Oct. 30, 1934 |
| 2,102,258 | Dornin        | Dec. 14, 1947 |
| 2,885,751 | Hornak et al. | May 12, 1959  |

#### FOREIGN PATENTS

|           |         |               |
|-----------|---------|---------------|
| 866,231   | Germany | Feb. 9, 1953  |
| 1,173,413 | France  | Oct. 27, 1958 |

#### OTHER REFERENCES

Gathmann: The Ingot Phase of Steel Production, pp. 30, 31, 1942.